

No. 813,453.

PATENTED FEB. 27, 1906.

C. R. SALMEN.

FIRE LIGHTING APPARATUS.

APPLICATION FILED SEPT. 23, 1905.



**WITNESSES**

Stuart W. Allen,  
William Armstrong.

**INVENTOR**

**CARL R. SALMEN.**

*By*  
Frank J. Lusk, A.T.Y.

# UNITED STATES PATENT OFFICE.

CARL RUDOLF SALMEN, OF MONTREAL, CANADA, ASSIGNOR OF ONE-FIFTH TO JOHN FISHER AND ONE-FIFTH TO FRANCIS SARLAY, OF CATA-SAUQUA, PENNSYLVANIA, ONE-FIFTH TO JOHN MRAZAY AND ONE-FIFTH TO EDWARD FIRNESZ, OF MONTREAL, CANADA.

## FIRE-LIGHTING APPARATUS.

No. 813,453.

Specification of Letters Patent.

Patented Feb. 27, 1906.

Application filed September 23, 1905. Serial No. 279,781.

*To all whom it may concern:*

Be it known that I, CARL RUDOLF SALMEN, of the city of Montreal, Province of Quebec, and Dominion of Canada, have invented certain new and useful Improvements in Fire-Lighting Apparatus, of which the following is a full, clear, and exact description.

My invention relates to a device for igniting fires; and the object is to provide a means by which wood, coal, or other fuel may be readily ignited with the least trouble and expense.

Referring to the drawing, the figure shows the preferred form of applying my device.

In the drawing, A represents a handle of wire or other suitable material.

B represents a frame, preferably of iron, inclosing a composition C, which is molded on the rod A. This composition consists of approximately thirty per cent. of finely-divided asbestos, approximately fifty per cent. of plaster-of-paris, ten per cent. graphite, and ten per cent. charcoal-dust. These proportions are mixed together with a small quantity of water and kneaded into a dough. The dough is then molded into a round or square brick and baked in an oven. During the process of baking it is brought to a red heat and emerges from the oven in a porous condition.

When it is desired to use the apparatus, it is soaked for a few minutes in kerosene or paraffin, with which it becomes impregnated. It may then be lighted and the fuel placed on top of it until ignition is sufficiently complete.

While I have stated the preferred proportions of ingredients constituting my invention, they may be varied within certain lim-

its. Moreover, the form of the igniter is immaterial, as I may use any other construction than that shown in the drawing.

Having thus described my invention so that the same may be readily understood by those skilled in the art to which it appertains, what I claim, and desire to secure by Letters Patent, is—

1. A device for lighting fires consisting of a composition of matter composed of, approximately, thirty per cent. finely-divided asbestos, fifty per cent. plaster-of-paris, ten per cent. graphite, and ten per cent. charcoal-dust.

2. A device for igniting fuel which consists of a composition of matter consisting of finely-divided asbestos, plaster-of-paris, graphite, and charcoal-dust, thoroughly mixed together, molded onto a suitable handle and baked, substantially as described.

3. A composition of matter for igniting fuel which consists of approximately one-third finely-divided asbestos, one-half plaster-of-paris, one-twelfth graphite, and one-twelfth charcoal-dust.

4. A device for igniting fuel comprising a composition of matter approximately thirty per cent. of asbestos, fifty per cent. plaster-of-paris, ten per cent. graphite, and ten per cent. charcoal-dust, kneaded into a dough, molded on a suitable handle, and afterward kiln-dried and impregnated with kerosene.

In witness whereof I have hereunto set my hand in the presence of two witnesses.

CARL RUDOLF SALMEN.

Witnesses:

WILLIAM G. ARMSTRONG,  
C. W. TAYLOR.